

Dec. 28, 1926.

1,612,776

L. KIRSCHBRAUN

ROOFING ELEMENT

Filed August 24, 1925

*fig. 1.*



*fig. 2.*



*fig. 3.*



*fig. 5.*



*fig. 6.*



*fig. 4.*



Inventor  
Lester Kirschbraun  
by  
Kirschbraun Murphy Day

Attns.

Patented Dec. 28, 1926.

1,612,776

# UNITED STATES PATENT OFFICE.

LESTER KIRSCHBRAUN, OF LEONIA, NEW JERSEY, ASSIGNOR TO THE FLINTKOTE COMPANY, OF BOSTON, MASSACHUSETTS, A CORPORATION OF MASSACHUSETTS.

## ROOFING ELEMENT.

Application filed August 24, 1925. Serial No. 51,949.

This invention relates to the production of roofing elements generally of the character of shingles, slabs, shingle strips, clapboard or the like, in which, when the material is laid upon the roof in overlapping courses, there are exposed marginal portions with edges that are subject to deterioration caused by the sunlight and the elements.

Ordinarily, in the manufacture of modern roofing such as employed for these purposes, it is the custom first to form a sheet of felt which is made ordinarily of rag fibers or rag and asbestos fibers or the like, of the desired caliper and of sufficient porosity to permit it to absorb a molten water-proofing composition such as pitch, asphalt or the like, and of sufficient strength to enable it to be manipulated during the operations of forming the ultimate roofing product. This is a common article of commerce which is ordinarily known as roofing felt and is produced on the usual paper-making machines. After the sheet has been properly saturated with the bituminous saturating compound, either by immersion in a bath of a molten bitumen or pitch, or by subjection to "pressure saturation", the sheet is coated on one face with a fairly thin layer of high melting point asphalt. For this purpose, oxidized or blown asphalt so-called is preferably employed because of its tough and rubbery nature. While the asphaltic coating is still soft and plastic and before it has set, it is surfaced with any suitable form of crushed mineral such as crushed slate, tile or any other mineral grit which will impart the desired color and texture to the final product. The grit is preferably formed in relatively large particles or granules which vary in form according to the material from which they are produced. The surface mineral coating is partially embedded in the plastic asphaltic coating sufficiently to insure a firm interlocking of the granules with the asphaltic coating, but leaving the granules so exposed that the asphaltic layer is completely covered and masked by the particles or grains of grit. In ordinary practice the sheet thus formed is now cut into roofing elements, which take the form of individual shingles or strip shingles or slabs of various designs or in long narrow strips which may be employed for the sides of buildings in the same manner as wooden clapboards.

The operation of the cutting machinery is

such that, when these roofing elements are produced, at all of the edges of the element there are exposed first the saturated felt, next a thin stratum of asphalt, and finally the layer of grit the grains of which are partially embedded in the asphalt.

It has been discovered that asphalt exposed to the elements and to the sunlight is susceptible to rapid deterioration. It is known, for example, that the action of sunlight or of the ultra violet rays is such as to cause a condensation or polymerization of the asphalt, resulting in the hardening of the asphalt with a consequent checking or breaking down of the asphalt particularly when it is exposed in relatively thin films or layers. This is especially true of the asphalt or other bitumen which is utilized as the saturating compound for the foundation felt, inasmuch as the films of asphalt about the fibers of the felt are relatively thin. Due to the action of the light and of moisture, these films crumble; and this, together with the absorption of moisture by the exposed fibers, causes the breaking down of the exposed edges and produces a tendency on the part of the exposed margin of the roofing element to curl. The curling is doubtless also accelerated by the fact that the layer of coating asphalt contracts under the influence of the elements and the rays of the sun and because of oxidation to a greater extent than the saturated felt itself.

On the other hand, a single layer of asphalt which is too thick is liable to crack through from internal stresses set up by unequal heating and cooling, especially in winter weather when the asphalt is comparatively hard and brittle. Cracks thus formed in a coating of asphalt admit moisture to the fibrous foundation of the element which is absorbed and tends to bulk or swell the felt. This, especially in conjunction with frost, tends to disintegrate the element by warping it, loosening the asphalt coating and extending the original crack or fissure. To secure best results in weather-proofing with a single coating of "blown" asphalt, such coating should be from .040 to .070 of an inch thick. The grit surfacing material usually applied to such a coating often comprises particles large enough to extend all the way through the coating and puncture it. If these particles are dislodged in the subsequent treatment and

handling of the roofing, they leave small pin-holes in the coating, through which moisture can enter. While these breaks in the continuity of the surface coat are not as serious a cause of deterioration of the element as are the cut exposed edges, yet their tendency is in the same direction, namely, to shorten the life of the element.

In the practical production of the roofing elements herein referred to, it is customary to apply the grit surface layer to only one face of the product, a portion of which is to be exposed to the weather, and in most cases the under face of the roofing elements consists of merely the saturated felt. In some instances it is true that a thin layer of the asphaltic coating is applied to the under face of the roofing element when the sheet is being saturated and coated. When the elements are laid in overlapping courses, however, water finds its way under the exposed edges and margins of the elements, either by capillary action or by the beating rain with the assistance of the wind, and in winter weather this moisture freezes and thaws and has the effect of lifting the exposed edges of the roofing elements from contact with the elements overlapped thereby, so that the deterioration of the asphalt hereinbefore referred to is localized not only at the edges of the roofing element but also extends through the under face thereof with the consequent tendency to disintegration and destruction of the foundation sheet. This is true even in cases where the under face of the product is coated, for the reason that ordinarily such coatings are so thin that they are rapidly attacked and their efficiency destroyed.

The problem which thus presents itself is to find some way of preventing or overcoming the deterioration at the cut edges of the roofing material and of prolonging the effective life of such roofing elements. In attacking this problem, one is confronted with the fact that the saturated felt is the weakest component of the roofing product so far as its liability to deterioration is concerned. The cellulosic fibers of which it is formed have an affinity for moisture, and the saturated felt itself ordinarily will absorb moisture up to 20% of its weight. Yet the integrity and the strength of the roofing product are directly dependent upon the integrity and strength of the saturated felt, for if this be destroyed the product as a whole loses its waterproofing and durable characteristics. The deterioration of the saturated felt is evidenced by progressive loss of cohesiveness and structural strength, so that the resistance of the final product to the weaving of the roof structure and its flexing through the action of the winds and the elements becomes insufficient to maintain it in place.

In seeking an answer to the problem,

therefore, means must be provided for the maximum protection of the saturated felt to prevent access of moisture, oxygen and light thereto. This is accomplished by providing what may be termed a supplemental coating of high melting point asphalt, preferably blown asphalt, in a layer of sufficient thickness so as completely to seal the fibers of the felt with an impermeable envelope so as to prevent the access of air or moisture; but, inasmuch as asphalt itself is subject to deterioration through the action of light as hereinbefore stated, the impermeable asphaltic envelope itself is liable to deterioration and destruction. Consequently to overcome this defect, means must be afforded for preventing the access of light to the asphaltic layer. This is accomplished by enclosing the asphaltic layer within an opaque layer. Any suitable opaque material may be utilized for this purpose, but as a practical matter one may employ crushed slate, crushed tile, or any other opaque granular material which may be partially embedded in the asphaltic layer in such manner as completely to cover it and to prevent the access of the rays of the sun directly thereto to any substantial extent.

The present invention comprises an individual roofing element in the nature of a shingle, shingle slab or strip, having the exposed edges sealed by an enclosing envelope of asphalt or bitumen and the envelope itself is protected against light by a surface layer of an opaque material preferably applied in granular form.

Incidentally, however, I have found that it is possible to produce a roofing material which is superior to those heretofore made of flat sheets, in that the element may be so formed that it is gradually thickened towards what may be called the butt or exposed end thereof. Thus, when the roofing elements are laid in overlapping courses, the roof thus formed has the appearance of and has an actual degree of thickness which imparts a pleasing effect and which relieves such roofs from the monotony and flatness that have characterized roofs formed of flat elements.

A roofing element thus formed possesses certain other highly desirable characteristics which are lacking in the ordinary flat element as heretofore produced. First, by reason of the fact that the element is thickest at the butt or exposed edge thereof, its weight is greatest at the edge and consequently the exposed edge offers greater resistance to the lifting force of the wind and will remain flat when the flat elements of unvarying thickness would be lifted or raised by the wind's pressure. This also permits of greater area of exposure. Again, inasmuch as both faces (that is, the upper and the lower faces) of the element are coated to

substantially the same extent by the asphaltic envelope, there is no tendency for the exposed portion of the element to curl away from the element overlapped thereby. Asphalt, when exposed to light and the elements, tends to contract; and, where the roofing element has no or only a thin layer of asphalt on its under side and a relatively thick layer on its exposed side, the contraction of the exposed layer causes the curling of the entire element. This is observable on many roofs which have been covered with flat individual slate-surfaced shingles.

Furthermore, an extra coating of asphalt over the surface of the element which is exposed when laid closes all pin holes and other possible breaks in the first coating which may occur by reason of punctures therethrough by particles of grit or in any other way, and although the second coating infiltrates between the particles of grit and bonds with the first coating, the grit layer maintains the separate identity of the two coatings and prevents the cracking stresses which would ordinarily be set up by thermal changes in a single layer of coating material of a thickness equal to the sum of the two coatings.

In the production of such elements as herein described, one may start with the ordinary roofing elements of commerce, namely, individual single shingles, strip shingles or slabs, or clapboard slabs, all of which are designed to be laid in overlapping courses with what may be termed for convenience exposed butt portions. These butt portions are dipped into a bath of molten asphalt for a sufficient time to cause them to be covered on both faces and on their exposed edges with a fairly thick layer of asphalt. By reference to Figures 3, 5 and 6 of the drawing, it will be seen that the coating around the butt edge of the shingle is rounded and of a substantial thickness. This is for the purpose of providing a surface free of sharp corners and with sufficient coating over the corners of the foundation to retain firmly grit which is thereafter applied. Furthermore, this enlarged rounded surface gives the shingle a very pleasing appearance. On removing the elements from the asphaltic bath, they are permitted to hang vertically and drain sufficiently to permit the excess asphalt to drop therefrom and to permit a flow of the attached coating so that it is thickest at the pendent edge of the element. While the coating is still soft and plastic, it is coated on both faces and on its edges with a layer of opaque granular material, the grains of which are partially embedded in the asphaltic coating but protrude therefrom so as to completely cover and mask the asphaltic envelope.

This process for treating pre-cut strip

shingles, which amounts to a refinishing of the portion of each strip which is to be exposed when laid, results in a very considerable saving in the roofing industry since it practically eliminates the waste due to "factory seconds," that is, finished elements which have slight defects which impair their salability and greatly reduce their value. The disposition of such elements has been a difficult problem involving considerable loss to manufacturers. By my invention, "seconds" can be reclaimed by the provision of the refinishing enveloping coat of asphalt and grit, and thus be made not only into a salable product, but one which is more durable and more effective and ornamental as a roof covering than the ordinary grit-surfaced shingles.

On the accompanying drawing I have illustrated a strip shingle embodying the invention, but it will be understood that the invention may equally well be incorporated or embodied in an individual single shingle, or an individual clapboard strip.

Fig. 1 represents a shingle strip as ordinarily formed, and which in the present instance serves as the starting material of my product;

Fig. 2 represents the completed product;  
Fig. 3 represents a section on the line 3-3 of Fig. 2;

Fig. 4 represents an enlarged section on line 4-4 of a part of the strip shingle;

Figs. 5 and 6 illustrate the formation of a double-dipped shingle.

Referring to the drawing, I have shown in Fig. 1, at *a* what is commercially known as a slate surfaced square butt strip shingle, which is provided at *b*, *b* with tabs or projections and intervening notches *c*, *c*. Such a shingle is usually laid with others in overlapping courses, so that the butts of the tabs register with the upper ends of the notches of the strips overlaid thereby. The tabs may, for example, be four inches in length, where the entire strip is ten inches between its upper and lower edges. Of course it will be understood that the design of the strip shingle may be varied, so that the tabs may be semi-hexagonal, or semi-octagonal, or of any other desired shape.

The shingle strip, as shown, has a base of rag or asbestos felt 10, which is impregnated with asphalt or other commonly used waterproofing compound, a layer 11 of higher melting point asphalt, and a surface layer 12 of granular material.

The strip is held by its straight upper edge, and is dipped into a bath of molten asphalt, which is preferably oxidized or blown asphalt having a melting point of 220°-240° F. The dipping operation must be carried on while the molten asphalt is at an elevated temperature, and is so timed that the strip will pick up the proper amount of

asphalt and also readily free itself of the excess. If a heavy coating is desired, the temperature of the bath is lower than when a thinner coating is to be applied. I have found that the desirable temperature to produce the optimum viscosity of the asphalt is in the range of 425°-450° F. when using oxidized asphalt from Mexican stock. It will be appreciated that the viscosity of an oxidized asphalt at a given temperature, will vary with the nature of the stock from which it is prepared, as well as its melting point, and the temperature to which it is heated. Therefore the temperature range which I have given is only indicative of the viscosity of the particular stock there referred to. The period in which a part of the shingle strip is dipped in the asphalt must be very short in order not to melt or unduly heat or soften the underlying bituminous material unnecessarily. One or two seconds is usually sufficient.

The shingle strip is dipped in the bath far enough to cause the molten asphalt to cover all of that portion of the strip which will be exposed when it is laid, usually to a longitudinal line parallel to the upper edge of the strip about half an inch to an inch above the ends of the notches. The strip is removed from the bath and while hanging is permitted to drain momentarily to permit the coating on both faces to flow toward the lower edge, and thus form tapered layers which are thickest at the edge, the excess drops being "flipped" or else wiped off. The strip is now surfaced with an opaque grit which is caused to become partially embedded in the still plastic asphaltic coating or envelope, not only on the faces of the strip but on all the edges thereof which are asphalt-coated, and as a consequence there is a continuous layer of exposed grit which extends over both faces and across all of the lower edges of the strip, including the edges of the tabs and the edges at the upper ends of the cutouts or notches. This may be done by first pressing the strip flatwise against a thick layer of loose grit, then rocking the strip through an arc of 180° about its asphalt-coated lower edge as the center, and pressing the other face against the layer of loose grit, and forcing or piling grit into the cut-outs or recesses and against the end edges of the strip. This molds the asphalt and grit at the lower edge of the strip and furnishes a straight rounded edge which is pleasing in appearance. The strips are piled one on the other, as produced, and the weight of the pile forms flat surfaces on the faces of the strips. The operations may, however, be performed by suitable automatic machinery.

In Fig. 2 of the drawing, I have shown the slate-surfaced strip shingle of Fig. 1, as it appears when it has been subjected to the

operations herein described. It will be noted from the sectional view illustrated by Fig. 3, that the shingle strip is thickest at its butt or lower edge, and tapers upwardly to a line just above the cut-outs or recesses. 70

In some cases for the opaque granular material, which is employed to cover, protect and mask the asphaltic envelope, I prefer to employ grit or granules of a different color and/or size from those which originally formed the outer layer of the original strip, especially in the case of strip shingles or individual shingles, so that a contrast will be afforded between the exposed portions thereof and the upper portions of the overlapped strips, which are visible through the notches, or through the spaces between the individual shingles. Again, instead of starting with a grit-coated roofing element, as hereinbefore described, one may start with a roofing element cut from "rubber roofing", so-called, which is an asphalt-impregnated sheet, having layers of high melting point asphalt on one or both faces thereof. Usually, but not necessarily, such "rubber roofing" has a surface layer of talc or mica. 85

I should not regard it as a departure from my invention if the protecting asphaltic envelope of the roofing elements were surfaced with pulverized material, or with talc or mica, or if the envelope itself were formed of a colorable pitch such as stearin pitch, or mixtures of resins and tempering fluxes, with a suitable pigment incorporated therein to impart the desired color thereto. 100

In instances where it is desired to keep down the weight of the roofing element, the front face and the edges of the strip may be surfaced with crushed slate partially embedded in the asphaltic envelope, and the rear face surfaced with a fine powder such as talc or mica. 105

In certain cases where an extra thick butt is desired on the roofing element, I may subject the element to a series of dipping and grit-surfacing operations. In such case, in the first dipping the element may be immersed, say, one and one half to two inches, and after the grit-surfacing operation has been carried out, and the asphaltic coating has set, the element is, in the second dipping immersed to an extent of five inches, after which it is surfaced, covered and protected with a layer of granules of opaque material. 115

In Figs. 4, 5 and 6, I have shown a strip which has been subjected to the series of operations last described.

In order to secure certain results, one may surface the edges of the cut-outs or recesses of a shingle strip with "fines" of the same color as the granules which coat the faces of the strip. Such "fines" are the powders or dusts which separate from the larger granules of slate or other mineral grit. 125 130

in each of the roofing elements herein described, the continuous asphaltic coating which covers the upper and under faces and the bottom and side edges of the exposed or butt portion thereof, is securely interlocked with the usual granular facing, if there be one, on the upper face of the element, and more or less coalesces with the asphaltic impregnating compound at the edges and on the underface of said butt portion. While the period of immersion or dipping is very short so as not to melt such impregnating compound and the initial asphaltic coating, yet there is sufficient heat in the second or continuous coating to cause a sufficient softening thereof and to cause the necessary coalescence and interlocking of the two.

The word "felting" as used in the specification and claims is intended to distinguish from a naturally formed fibrous structure such as wood but is used with a view of including any base made from segregated fibres formed into a sheet, or base of an equivalent nature, by any suitable machinery.

Having thus explained the nature of my improvements and a mode of producing products embodying the same, what I claim is:

1. A roofing element adapted to be laid with others in overlapping courses comprising a felted foundation impregnated with a waterproofing material, a coating of asphalt on the exposed face, the butt and side edges and a portion of the under face thereof, and a surface layer of granular material partially embedded in the asphalt coating extending over the said exposed and under face of the element and the butt edges thereof.

2. A flexible roofing element adapted to be laid with others in overlapping courses comprising a flexible felted foundation impregnated with a waterproofing material, a continuous envelope of asphalt encasing the exposed face, the butt and side edges and a portion of the under face thereof, and a surface layer of granular material partially embedded in the asphalt coating extending over the said exposed and under face of the element and the butt and side edges thereof.

3. A roofing element adapted to be laid with others in overlapping courses comprising a felted foundation impregnated with a waterproofing material, a coating of asphalt on the exposed face, butt and side edges and a portion of the under face thereof, a surface layer of granular material partially embedded in said asphalt coating extending over the exposed face of the element and the butt and side edges thereof, and a layer of comminuted material partially embedded in the asphalt coating on the under face of said element.

4. A flexible roofing element adapted to be laid with others in overlapping courses, comprising a saturated flexible fibrous founda-

tion, a coating of asphalt thereon covering the exposed face of the element when laid, the butt and side edges and a portion of the under face thereof, said coating extending over the butt edge being substantially round, 70 and a surface layer of granular material partially embedded in said asphalt coating on the faces of the element and in the rounded coating extending around the butt edge thereof. 75

5. A roofing element adapted to be laid with others in overlapping courses comprising a saturated felted foundation, a coating of asphalt thereon covering the exposed faces of the element when laid, the butt and side edges and a portion of the under face thereof, said coating extending over the butt edge being substantially rounded and a surface layer of granular material partially embedded in said asphalt coating on the exposed face and side edges of the element and in the rounded coating extending around the butt edge thereof. 85

6. A roofing element adapted to be laid with others in overlapping courses comprising a felt foundation impregnated with a bitumen coating of asphalt thereon covering the exposed face of the element when laid, the butt and side edges and a portion of the under face thereof, said coating being thickened and rounded about said butt edge, and a surface layer of granular material partially embedded in said asphalt coating on the exposed face and the side edges thereof and in the thickened rounded coating extending 95 around the butt edge thereof. 100

7. An individual roofing element adapted to be laid with others in overlapping courses, comprising a flexible fibrous foundation impregnated with asphalt, and having its upper face thereof coated with asphalt and surfaced with a comminuted material, said element having an additional and continuous asphaltic envelope extending over that portion of the upper face of the element 110 which is exposed when said element is laid as described, over the bottom and side edges and over a portion of the under face of said element, whereby all of the exposed portions of said element are encased within a continuous waterproof coating of asphalt and a layer of comminuted mineral embedded in said asphalt coating on the upper exposed face of said element. 115

8. An individual roofing element adapted to be laid with others in overlapping courses, comprising a flexible felted foundation impregnated with asphalt, and having its upper face thereof coated with asphalt and surfaced with partially embedded grit, said element having an additional and continuous asphaltic envelope extending over that portion of the upper face of the element which is exposed when said element is laid as described, over the bottom and side edges, 130

and over a portion of the under face of said element, whereby all of the exposed portions of said element are encased within a continuous waterproof coating of asphalt, and 5 a layer of granular material partially embedded in said envelope on the upper face and on the bottom and side edges thereof.

9. An individual roofing element adapted to be laid with others in overlapping courses, 10 said element comprising the usual grit-surfaced asphalt-coated waterproof felted foundation, and having in addition a continuous coating of asphalt superimposed upon the butt portions of the upper and under faces 15 and the intermediate edge portions thereof, and a layer of granular material partially embedded in and masking said asphaltic coating, said coating of asphalt and layer of granular material being thickest at the butt 20 edge of said element.

10. An individual roofing element adapted to be laid with others in overlapping courses, said element comprising the usual grit-surfaced asphalt-coated waterproof felted foundation, and having in addition a continuous coating of asphalt superimposed upon the butt portions of the upper and under faces and the intermediate edge portions 25 thereof, and a layer of granular material

partially embedded in and masking said asphaltic coating, said coating of asphalt and layer of granular material being thickest at the butt edge of said element and being rounded about said butt edge. 30

11. A shingle strip having a plurality of tabs with intervening recesses and adapted to be laid with others in overlapping courses with the tabs exposed in simulation of shingles or tiles, said strip comprising an asphalt-impregnated fibrous foundation having on its upper face a coating of asphalt with a surface layer of grit partially embedded therein, and also having in addition a continuous external coating of asphalt covering the upper and under faces of the tabs and the side and bottom edges thereof, and an external surface layer of granular material partially embedded in and covering said continuous asphaltic coating, said continuous asphaltic coating and surface layer 40 being thickest at the butt edge of said element and tapering toward and terminating at a line parallel with the top edge and above but adjacent to the upper ends of said recesses. 45

In testimony whereof I have affixed my signature.

LESTER KIRSCHBRAUN. 50